



US010455643B2

(12) **United States Patent**  
**Huang**

(10) **Patent No.:** **US 10,455,643 B2**  
(45) **Date of Patent:** **Oct. 22, 2019**

(54) **THICK FILM ELEMENT HAVING  
COVERING LAYER WITH HIGH HEAT  
CONDUCTIVITY**

(71) Applicant: **GUANGDONG FLEXWARM  
ADVANCED MATERIALS &  
TECHNOLOGY CO., LTD.,**  
Guangzhou, Guangdong (CN)

(72) Inventor: **Weicong Huang**, Guangdong (CN)

(73) Assignee: **GUANGDONG FLEXWARM  
ADVANCED MATERIALS &  
TECHNOLOGY CO., LTD.,**  
Guangzhou, Guangdong (CN)

(\*) Notice: Subject to any disclaimer, the term of this patent is extended or adjusted under 35 U.S.C. 154(b) by 0 days.

(21) Appl. No.: **15/534,487**

(22) PCT Filed: **Mar. 26, 2016**

(86) PCT No.: **PCT/CN2016/077441**

§ 371 (c)(1),  
(2) Date: **Jun. 9, 2017**

(87) PCT Pub. No.: **WO2017/133069**

PCT Pub. Date: **Aug. 10, 2017**

(65) **Prior Publication Data**

US 2018/0352609 A1 Dec. 6, 2018

(30) **Foreign Application Priority Data**

Feb. 3, 2016 (CN) ..... 2016 1 0076006

(51) **Int. Cl.**

**H05B 3/12** (2006.01)  
**H05B 3/02** (2006.01)  
**H05B 3/22** (2006.01)  
**H05B 3/34** (2006.01)  
**F28F 3/04** (2006.01)

(52) **U.S. Cl.**

CPC ..... **H05B 3/12** (2013.01); **F28F 3/04**  
(2013.01); **H05B 3/02** (2013.01); **H05B 3/22**

(2013.01); **H05B 3/34** (2013.01); **H05B  
2203/01** (2013.01); **H05B 2203/013** (2013.01)

(58) **Field of Classification Search**  
CPC ..... H05B 3/262; H05B 3/748; H05B 3/82;  
H05B 3/12; H05B 3/02; H05B 3/22;  
H05B 3/34; H05B 3/26; H05B 3/265;  
H05B 3/267; H05B 2203/013; H05B  
2203/017; H05B 2203/037; H05B  
2203/01

See application file for complete search history.

(56) **References Cited**

FOREIGN PATENT DOCUMENTS

|    |           |        |
|----|-----------|--------|
| CN | 103140721 | 6/2013 |
| CN | 103744276 | 4/2014 |
| GB | 9703225D0 | 4/1997 |

Primary Examiner — Shawntina T Fuqua

(57) **ABSTRACT**

The present invention provides a thick film element having a covering layer with high heat conductivity, which comprises a carrier, a thick film coating deposited on the carrier and a covering layer overlaid on the coating. The thick film coating is a heating materials, and the mode of heating is electrical heating. The covering layer, the thick film coating and the carrier are selected from a material that fulfills every of the following equations:

$$\lambda_1 A \frac{T_1 - T_0}{d_1} = a \times \lambda_3 A \frac{T_3 - T_0}{d_3},$$

$$\lambda_2 A \frac{T_2 - T_0}{d_2} = b \times \lambda_1 A \frac{T_1 - T_0}{d_1},$$

$$\lambda_2 A \frac{T_2 - T_0}{d_2} = c \times \lambda_3 A \frac{T_3 - T_0}{d_3};$$

wherein  $200 \leq a \leq 10^4$ ,  $0 < b \leq 1000$ ,  $0 < c \leq 5 \times 10^5$ . The covering layer of the thick film element of the present invention has high heat conductivity, and is suitable for coating products with a single-sided heating covering layer. The present invention improves heat transfer efficiency and reduces heat loss when double-sided heating is not required.

**16 Claims, No Drawings**

## THICK FILM ELEMENT HAVING COVERING LAYER WITH HIGH HEAT CONDUCTIVITY

### FIELD OF THE INVENTION

The present invention relates to the field of thick film, and more particularly to a thick film element having a covering layer with high heat conductivity.

### BACKGROUND OF THE INVENTION

Thick film technology was developed in the 1960s and is widely used in many industries after several decades of development. However, the development of thick film heating technology is not long. Thick film heating elements refer to heating elements that are made by fabricating exothermic materials on a substrate into thick films and providing electricity thereto to generate heat. The conventional heating methods include electrical heated tube heating and PTC heating. Both methods adopt indirect heating. Both electrical heated tube heating and PTC heating conduct heat indirectly with low thermal efficiency, and are structurally huge and bulky. Besides, in consideration of environmental protection, heaters using these two types of heating methods stain easily after repeatedly heating and cleaning thereof is not easy. Additionally, PTC heaters contain lead and other hazardous substances and are easily oxidized, causing power attenuation and short service life.

Chinese application CN2011800393787 discloses a combination of an electrical heating element and a heat dissipator heated thereby. The heating element comprises a substrate, an insulating layer located on the substrate and a thick film conductor located on the insulating layer; wherein the second side of the metallic substrate is in contact with the heat dissipator, which comprises a layer of metallic material on a surface thereof facing the heater. The substrate is brazed to the heat dissipator, and the surface of the heating element over which the thick film conductor extends is substantially equal to the surface of the heat dissipator.

It could be seen from the above technology that the thick film technology is developing gradually; however, the thick film conductors of the above-mentioned thick film heating element are combined with the substrate through the insulating layer, instead of coated on the substrate directly. Such heating element could not transfer heat to the substrate directly when the thick film is given electricity to generate heat, which would affect the heat generating rate. Besides, the above technical solution overcomes heat dissipation problem of the thick film by utilizing external devices, but does not provide solutions in designing thick film elements of specific materials for various products to solve heat dissipation problem caused by excess heating temperature of the thick films. There are few thick film heating products that could realize direct heating, especially for situations in which heating of only a single side is required. The application of a thick film circuit for single-side heat transferring covering layer in the products to transfer heat only on one side to reduce heat loss has greatly broaden the development of heating products. The existing heating devices could meet the demands of heating; however, heating device that performs unilateral heating transfer is rarely seen, or unilateral heat transfer of such device is too poor, making it difficult to reduce heat loss by keeping high unilateral thermal conduction properties.

### SUMMARY OF THE INVENTION

To solve these problems mentioned above, the present invention provides a thick film element having a covering

layer with high heat conductivity that has the advantages of small volume, high efficiency, environmental-friendly, high safety performance and long service lifespan.

The concept of thick film in the present invention is a term comparative to thin films. Thick film is a film layer with a thickness ranging from several microns to tens of microns formed by printing and sintering on a carrier; the material used to manufacture the film layer is known as thick film material, and the coating made from the thick film is called thick film coating. The thick film element has the advantages of high power density, fast heating speed, high working temperature, fast heat generating rate, high mechanical strength, small volume, easy installation, uniform heating temperature field, long lifespan, energy saving and environmental friendly, and excellent safety performance.

The thick film element having a covering layer with high heat conductivity of the present invention, comprises a carrier, a thick film coating deposited on the carrier and a covering layer overlaid on the coating. The thick film coating is a heating material, and the mode of heating is electrical heating. The carrier, the thick film coating and the covering layer are selected from a material that fulfills every of the following equations:

$$\begin{aligned} \lambda_1 A \frac{T_1 - T_0}{d_1} &= a \times \lambda_3 A \frac{T_3 - T_0}{d_3}, \\ \lambda_2 A \frac{T_2 - T_0}{d_2} &= b \times \lambda_1 A \frac{T_1 - T_0}{d_1}, \\ \lambda_2 A \frac{T_2 - T_0}{d_2} &= c \times \lambda_3 A \frac{T_3 - T_0}{d_3}; \\ 200 \leq a \leq 10^4, 0 < b \leq 1000, 0 < c \leq 5 \times 10^5; \end{aligned}$$

$T_2 < T_{\text{Minimum melting point of the covering layer}}$ ;  
 $T_2 < T_{\text{Minimum melting point of the carrier}}$ ;  
 $T_0 \leq 30^\circ \text{C.}$ ;  
 wherein the value of

$$\lambda_1 A \frac{T_1 - T_0}{d_1}$$

represents the heat transfer rate of the covering layer; the value of

$$\lambda_2 A \frac{T_2 - T_0}{d_2}$$

represents the heating rate of the thick film coating; the value of

$$\lambda_3 A \frac{T_3 - T_0}{d_3}$$

represents the heat transfer rate of the carrier;  
 $\lambda_1$  represents the heat conductivity coefficient of the covering layer at the temperature of  $T_1$ ;  $\lambda_2$  represents the heat conductivity coefficient of the thick film coating at the temperature of  $T_2$ ;  
 $\lambda_3$  represents the heat conductivity coefficient of the carrier at the temperature of  $T_3$ ;

A represents the contact area of the thick film coating with the covering layer or the carrier;  
 $d_1$  represents the thickness of the covering layer;  
 $d_2$  represents the thickness of the thick film coating;  
 $d_3$  represents the thickness of the carrier;  
 $T_0$  represents the initial temperature of the thick film element;  
 $T_1$  represents the surface temperature of the covering layer;  
 $T_2$  represents the heating temperature of the thick film coating;  
 $T_3$  represents the surface temperature of the carrier;  
 $d_2 \leq 50 \mu\text{m}$ ;  
and  $10 \mu\text{m} \leq d_1 \leq 10 \text{ mm}$ ,  $d_3 \geq 10 \mu\text{m}$ ;  
 $T_{\text{Minimum melting point of the carrier}} > 25^\circ \text{C}$ ;  
 $\lambda_1 \geq \lambda_3$ ;

the covering layer is a dielectric layer covering on the thick film coating by printing or sintering, and the area of the covering layer is larger than that of the thick film coating.

The carrier is the dielectric layer carrying the thick film coating. The thick film coating covers the carrier by printing or sintering, and is the coated substrate of the thick film element.

The heat conductivity coefficient refers to the heat transferred by a one-meter thick material having a temperature difference between two side surfaces of 1 degree (K, °C.), through one square meter ( $1 \text{ m}^2$ ) area within one second (1 S) under a condition of stable heat transfer. Unit of the heat conductivity coefficient is watt/meter·degree (W/(m·K)), and K may be replaced by °C.).

The covering layer, the thick film coating and the carrier stick closely with each other at the electrical heating parts of the thick film elements, and both sides of the thick film coating connect to external electrodes. When given electricity, the thick film coating is heated and becomes hot after electricity energy is transformed to thermal energy. Heat generating rate of the thick film coating could be calculated by

$$\lambda_2 A \frac{T_2 - T_0}{d_2}$$

according to the heat conductivity coefficient, the contact area, initial temperature, heating temperature and thickness of the thick film coating, wherein  $T_2$  represents the heating temperature of the thick film.

The present invention features in that the thick film element has a covering layer with high heat conductivity, and that the heat generating rate of the covering layer, the carrier and the thick film coating should meet the following requirements:

(1) The heat transfer rate of the thick film coating and the covering layer should satisfy the following formula:

$$\lambda_1 A \frac{T_1 - T_0}{d_1} = a \times \lambda_3 A \frac{T_3 - T_0}{d_3},$$

wherein  $200 \leq a \leq 10^4$ ; for those thick film elements satisfied the above equation, the heat transfer capability of their covering layer is superior to that of the carrier, which means that the covering layer is fast while the carrier is slow at temperature rising or that the temperature difference between the covering layer and the carrier is large after stable heat balance. Therefore, the thick film elements generally show the technical effect of covering layer heating.

(2) The heat generating rate of the thick film coating and the heat transfer rate of the covering layer should satisfy the following formula:

$$\lambda_2 A \frac{T_2 - T_0}{d_2} = b \times \lambda_1 A \frac{T_1 - T_0}{d_1},$$

wherein  $0 < b \leq 1000$ ; if the heat generating rate of the thick film coating is much larger than that of the covering layer, the continuously accumulated heat of the thick film coating could not be conducted away, such that the temperature of the thick film coating keeps rising, and when the temperature is higher than the minimum melting point of the covering layer, the covering layer would begin to melt or even burn, which would destroy the structure of the covering layer or the carrier, thus destroying the thick film elements.

(3) The heat generating rate of the thick film coating and the heat transfer rate of the carrier should satisfy the following formula:

$$\lambda_2 A \frac{T_2 - T_0}{d_2} = c \times \lambda_3 A \frac{T_3 - T_0}{d_3}, \quad 0 < c \leq 5 \times 10^5;$$

since both the heat conductivity coefficient and heat transfer rate of the carrier is small, if the heat generating rate of the thick film coating is much larger than that of the carrier, the continuously accumulated heat of the thick film coating could not be conducted away, such that the temperature of the thick film coating keeps rising, and when the temperature is higher than the minimum melting point of the carrier, the carrier would begin to melt or with thermal deformation, or even start to burn, which would destroy the structure of the carrier, thus destroying the thick film elements.

(4) The heating temperature of the thick film coating could not be higher than the minimum melting point of the covering layer or the carrier, and should meet the requirements:  $T_2 < T_{\text{Minimum melting point of the covering layer}}$  and  $T_2 < T_{\text{Minimum melting point of the carrier}}$ . Excessively high heating temperature should be avoided to prevent destruction of the thick film elements.

When the above-mentioned requirements are met, the heat transfer rate of the covering layer and the carrier is determined by the properties of the material and the thick film element:

The formula for calculating the heat transfer rate of the covering layer is

$$\lambda_1 A \frac{T_1 - T_0}{d_1},$$

wherein  $\lambda_1$  represents the heat conductivity coefficient of the covering layer, with the unit being W/m·K, and is determined by properties of the materials for preparing the covering layer;  $d_1$  represents the thickness of the covering layer, and is determined by the preparation technique and the requirements of the thick film elements;  $T_1$  represents the surface temperature of the covering layer, and is determined by the properties of the thick film elements.

The formula for calculating the heat transfer rate of the carrier is

$$\lambda_3 A \frac{T_3 - T_0}{d_3},$$

wherein  $\lambda_3$  represents the heat conductivity coefficient of the carrier, with the unit being W/m·k, and is determined by properties of the materials for preparing the carrier;  $d_3$  represents the thickness of the carrier, and is determined by the preparation technique and the requirements of the thick film elements;  $T_3$  represents the surface temperature of the carrier, and is determined by properties of the thick film elements.

Preferably, the heat conductivity coefficient of the carrier  $\lambda_3$  is  $\leq 3$  W/m·k, the heat conductivity coefficient of the covering layer is  $\lambda_1 \geq 3$  W/m·k; wherein  $200 \leq a \leq 10^4$ ,  $10 \leq b \leq 1000$ ,  $10^4 \leq c \leq 5 \times 10^5$ .

Preferably, the carrier and the thick film coating is bound by printing or sintering; the thick film coating and the covering layer is bound by printing, sintering, or vacuum.

Preferably, the region between the carrier and the covering layer without the thick film coating is bound by printing, coating, spraying or sintering, or with gluing.

Preferably, the carrier includes polyimides, organic insulating materials, inorganic insulating materials, ceramics, glass ceramics, quartz, stone materials, fabrics and fiber.

Preferably, the thick film coating is one or more of silver, platinum, palladium, palladium oxide, gold and rare earth materials.

Preferably, the covering layer is made from one or more of polyester, polyimide or polyetherimide (PEI), ceramics, silica gel, asbestos, micarex, fabric and fiber.

Preferably, the area of the thick film coating is smaller than or equal to the area of the covering layer or the carrier.

The present invention also provides a use of the thick film elements for coating products with covering layer heating.

The beneficial effects of the present invention are as follows:

(1) The covering layer of the thick film element of the present invention has high heat conductivity, and is suitable for coating products with covering layer heating to improve heat transfer efficiency and reduce heat losses when double-sided heating is not required. The covering layer of the present invention is suitable for thick film elements having a carrier that could be coated with a thick film but has a small heat conductivity coefficient. The covering layer of the present invention has high heat conductivity and could achieve single-sided heat transferring effects.

(2) The three-layered structure of the thick film element of the present invention could be bound directly by printing or sintering, and the thick film coating would heat the covering layer directly without the need of any medium. Hence, heat could be conducted to the covering layer directly, thus improving heat conduction efficiency. Additionally, the covering layer of the present invention is overlaid on the thick film coating, avoiding electric leakage of the thick film coating after given electricity and improving safety performance.

The thick film element of the present invention generates heat by the thick film coating, the thickness ranges of which is at the micrometer level, and has a uniform heat generating rate and long service lifespan.

#### DETAILED DESCRIPTION OF PREFERRED EMBODIMENTS

The present invention will now be described more specifically with reference to the following embodiments. It is

to be noted that the following descriptions of preferred embodiments of this invention are presented herein for purpose of illustration and description only. It is not intended to be exhaustive or to be limited to the precise form disclosed.

The present invention discloses a thick film element having a covering layer with high heat conductivity, which comprises a carrier, a thick film coating deposited on the carrier and a covering layer overlaid on the coating; the thick film coating is a heating material, and the mode of heating is electrical heating, wherein the carrier, the thick film coating and the covering layer are selected from a material that fulfills every of the following equations:

$$\begin{aligned} 15 \quad \lambda_1 A \frac{T_1 - T_0}{d_1} &= a \times \lambda_3 A \frac{T_3 - T_0}{d_3}, \quad \lambda_2 A \frac{T_2 - T_0}{d_2} = b \times \lambda_1 A \frac{T_1 - T_0}{d_1}, \\ 20 \quad \lambda_2 A \frac{T_2 - T_0}{d_2} &= c \times \lambda_3 A \frac{T_3 - T_0}{d_3}; \\ 25 \quad 200 \leq a \leq 10^4, 0 < b \leq 1000, 0 < c \leq 5 \times 10^5; \end{aligned}$$

$T_2 < T_{\text{Minimum melting point of the covering layer}}$ ;

$T_2 < T_{\text{Minimum melting point of the carrier}}$ ;

$T_0 \leq 30^\circ \text{ C.}$ ;

$d_2$  represents the thickness of the thick film coating,  $d_2 \leq 50 \mu\text{m}$ ;

and  $10 \mu\text{m} \leq d_1 \leq 10 \text{ mm}$ ,  $d_3 \geq 10 \mu\text{m}$ ;

$T_{\text{Minimum melting point of the carrier}} > 25^\circ \text{ C.}$ ;

$\lambda_1$  represents the heat conductivity coefficient of the covering layer,  $\lambda_3$  represents the heat conductivity coefficient of the carrier, and  $\lambda_1 \geq \lambda_3$ .

The following embodiments includes 20 thick film elements prepared by the inventors, and the materials for preparing the covering layer, the thick film coating and the carrier of the 20 listed thick film elements all satisfy the equations above. The detailed preparing method and formula are provided as follows:

#### Embodiments

Silver paste with a heat conductivity coefficient of  $\lambda_2$  is selected to prepare the thick film coating, polyimides with a heat conductivity coefficient of  $\lambda_3$  is selected to prepare the carrier, and polyimides with a heat conductivity coefficient of  $\lambda_1$  is selected to prepare the covering layer. The three layer are bound by sintering. The area of the prepared thick film coating is  $A_2$ , the thickness is  $d_2$ ; the area of the covering layer is  $A_1$ , the thickness is  $d_1$ ; the area of the carrier is  $A_3$ , the thickness is  $d_3$ .

Turn on an external DC power supply to charge the thick film coating. The thick film starts to heat up; when the heating is stabled, measure the surface temperature of the covering layer and the carrier, and the heating temperature of the thick film coating under a stable heating state are measured. Heat transfer rate of the covering layer and the carrier, and heat generating rate of the thick film coating are calculated according to the following formula:

$$60 \quad \lambda_1 A \frac{T_1 - T_0}{d_1}, \quad \lambda_2 A \frac{T_2 - T_0}{d_2}, \quad \lambda_3 A \frac{T_3 - T_0}{d_3}.$$

Tables 1 to 4 are the 20 thick film elements prepared by the inventors. After provided electricity to heat for 2 minutes, the thick film elements are measured according the national standards to obtain the performance data (heat

conductivity coefficient, surface temperature) as shown in the Tables. The thickness, contact area, initial temperature are measured before heating.

The methods to measure the heat conductivity coefficient of the covering layer, the thick film coating and the carrier are as follows:

(1) Switch on the power and adjust the heating voltage to a specified value, turn on the power switch of the device with 6V power and preheat for 20 minutes;

(2) Conduct zero calibration for the light spot galvanometer;

(3) Calibrate the standard operating voltage of UJ31 potentiometer according to the room temperature, set the commutator switch of the potentiometer to a standard position and adjusts the operating current of the potentiometer; As the voltage of the standard batteries vary with the temperature, room temperature calibration is calculated by the following formula:

$$E_t = E_0 - [39.94(t-20) + 0.929(t-20)^2]; \text{ wherein } E_0 = 1.0186V.$$

(4) Place a heating plate and lower thermoelectric couples on the bottom part of the thin test specimen; place upper thermoelectric couples on the upper part of the thin test specimen. It should be noted that the thermoelectric couples must be placed at the central position of the test specimen, and cold sections of the thermoelectric couples must be placed in an ice bottle.

(5) Place the commutator switch of the potentiometer at the position 1, measure the initial temperatures at the upper part and the lower part of the test specimen; proceed only when the temperature difference between the upper part and the lower part is smaller than 0.004 mV (0.1° C.).

(6) Pre-add 0.08 mV to the initial thermoelectric potential of the upper thermoelectric couples, turn on the heating switch to start heating; meanwhile, watch the time with a stopwatch; when the light spot of a light spot galvanometer returns to zero position, turn off the heating source to obtain excess temperature and heating time of the upper part.

(7) Measure the thermoelectric potential of the lower thermoelectric couples after 4-5 minutes to obtain excess temperature and heating time of the lower part.

(8) Place the commutator switch of the potentiometer at the position 2, turn on the heating switch to measure the heating current.

(9) End the test, turn off the power and clear up the instrument and equipment.

The temperature is measured by using a thermo-couple thermometer as follows:

(1) Connect the thermo-sensing wires to the surfaces of the thick film coating, the carrier, and the covering layer of the heating elements, and the outdoor air.

(2) Provide electricity to the heating product with rated power, and measure the temperature of all parts.

(3) Record the temperature  $T_0, T_1, T_2, T_3$  at all parts of the products at every time interval by a connected computer.

The thickness is measured by using a micrometer and by piling up and averaging the values.

The method to measure the melting point is as follows:

The detection instrument: differential scanning calorimeter, model DSC2920, manufactured by TA Instruments (USA). The instrument is qualified (Level A) as verified by

20 Verification Regulation of Thermal Analyzer 014-1996.

(1) Ambient temperature: 20-25° C.; Relative humidity: <80%;

(2) Standard material for instrument calibration: Thermal analysis standard material—Indium, standard melting point 25 429.7485 K (156.60).

(3) Measuring procedure: referring to “GB/T19466.3—2004/ISO” for the detection procedure.

Repeat the measurement for three times to ensure normal operation of the instrument before sample testing: weight

30 1-2 mg of the sample, with an accuracy of 0.01 mg, place the sample in an aluminum sample plate. Testing conditions:

heat the sample to 200° C. at a rate of 10° C./min, and repeat the measurement for ten times. Measurement model: collect the information of melting points by the computer and

35 instrument, determine the initial extrapolated temperature of the endothermic melting peak by automatic collection of measured data and program analysis of spectra to directly obtain the measurement model. The measurement results are

calculated according to the Bessel formula.

40 Table 1 is the performance data of the covering layers of thick film elements in Embodiments 1 to 20. The details are as follows:

TABLE 1

|               | Covering Layer                                      |                      |                                 |                                                                |                                 |                                    |
|---------------|-----------------------------------------------------|----------------------|---------------------------------|----------------------------------------------------------------|---------------------------------|------------------------------------|
|               | Heat Conductivity Coefficient $\lambda_1$ (W/m · k) | Thickness $d_1$ (μm) | Surface Temperature $T_1$ (°C.) | $T_{\text{Minimum melting point of the covering layer}}$ (°C.) | Initial Temperature $T_0$ (°C.) | Heat Transfer Rate/10 <sup>6</sup> |
| Embodiment 1  | 7.22                                                | 200                  | 110                             | 350                                                            | 25                              | 0.036822                           |
| Embodiment 2  | 7.23                                                | 100                  | 110                             | 350                                                            | 25                              | 0.073746                           |
| Embodiment 3  | 7.24                                                | 80                   | 108                             | 350                                                            | 25                              | 0.090138                           |
| Embodiment 4  | 7.24                                                | 80                   | 102                             | 350                                                            | 25                              | 0.083622                           |
| Embodiment 5  | 7.24                                                | 60                   | 100                             | 350                                                            | 25                              | 0.0905                             |
| Embodiment 6  | 7.18                                                | 60                   | 98                              | 350                                                            | 25                              | 0.087356667                        |
| Embodiment 7  | 7.18                                                | 50                   | 102                             | 350                                                            | 25                              | 0.1548008                          |
| Embodiment 8  | 7.17                                                | 50                   | 100                             | 350                                                            | 25                              | 0.15057                            |
| Embodiment 9  | 7.23                                                | 40                   | 100                             | 350                                                            | 25                              | 0.1897875                          |
| Embodiment 10 | 7.23                                                | 40                   | 102                             | 350                                                            | 25                              | 0.167013                           |
| Embodiment 11 | 7.2                                                 | 40                   | 98                              | 350                                                            | 25                              | 0.15768                            |
| Embodiment 12 | 7.2                                                 | 35                   | 108                             | 350                                                            | 25                              | 0.204891429                        |
| Embodiment 13 | 7.15                                                | 35                   | 90                              | 350                                                            | 25                              | 0.159342857                        |
| Embodiment 14 | 7.15                                                | 35                   | 90                              | 350                                                            | 25                              | 0.212457143                        |
| Embodiment 15 | 7.16                                                | 30                   | 101                             | 350                                                            | 25                              | 0.290218667                        |
| Embodiment 16 | 7.24                                                | 30                   | 100                             | 350                                                            | 25                              | 0.181                              |
| Embodiment 17 | 7.24                                                | 30                   | 89                              | 350                                                            | 25                              | 0.262570667                        |
| Embodiment 18 | 7.17                                                | 25                   | 90                              | 350                                                            | 25                              | 0.223704                           |
| Embodiment 19 | 7.22                                                | 25                   | 94                              | 350                                                            | 25                              | 0.3188352                          |

TABLE 1-continued

| Covering Layer |                                                     |                      |                                  |                                                                 |                                  |                                    |
|----------------|-----------------------------------------------------|----------------------|----------------------------------|-----------------------------------------------------------------|----------------------------------|------------------------------------|
|                | Heat Conductivity Coefficient $\lambda_1$ (W/m · k) | Thickness $d_1$ (μm) | Surface Temperature $T_1$ (° C.) | $T_{\text{Minimum melting point of the covering layer}}$ (° C.) | Initial Temperature $T_0$ (° C.) | Heat Transfer Rate/10 <sup>6</sup> |
| Embodiment 20  | 7.22                                                | 20                   | 92                               | 350                                                             | 25                               | 0.314431                           |

Table 2 is the performance data of the thick film coatings of thick film elements in Embodiments 1 to 20. The details are as follows:

TABLE 2

| Thick Film Coating |                                                     |                      |                              |                                  |                                  |                                      |
|--------------------|-----------------------------------------------------|----------------------|------------------------------|----------------------------------|----------------------------------|--------------------------------------|
|                    | Heat Conductivity Coefficient $\lambda_2$ (W/m · k) | Thickness $d_2$ (μm) | Area $A_2$ (m <sup>2</sup> ) | Heating Temperature $T_2$ (° C.) | Initial Temperature $T_0$ (° C.) | Heat Generating Rate/10 <sup>6</sup> |
| Embodiment 1       | 385                                                 | 30                   | 0.012                        | 118                              | 25                               | 14.322                               |
| Embodiment 2       | 384                                                 | 30                   | 0.012                        | 116                              | 25                               | 13.9776                              |
| Embodiment 3       | 380                                                 | 30                   | 0.012                        | 112                              | 25                               | 13.224                               |
| Embodiment 4       | 382                                                 | 40                   | 0.012                        | 109                              | 25                               | 9.6264                               |
| Embodiment 5       | 382                                                 | 50                   | 0.01                         | 102                              | 25                               | 5.8828                               |
| Embodiment 6       | 385                                                 | 45                   | 0.01                         | 104                              | 25                               | 6.7588888889                         |
| Embodiment 7       | 385                                                 | 55                   | 0.014                        | 108                              | 25                               | 8.134                                |
| Embodiment 8       | 380                                                 | 35                   | 0.014                        | 112                              | 25                               | 13.224                               |
| Embodiment 9       | 382                                                 | 45                   | 0.014                        | 111                              | 25                               | 10.22062222                          |
| Embodiment 10      | 382                                                 | 40                   | 0.012                        | 118                              | 25                               | 10.6578                              |
| Embodiment 11      | 382                                                 | 35                   | 0.012                        | 106                              | 25                               | 10.60868571                          |
| Embodiment 12      | 380                                                 | 35                   | 0.012                        | 114                              | 25                               | 11.59542857                          |
| Embodiment 13      | 380                                                 | 20                   | 0.012                        | 108                              | 25                               | 18.924                               |
| Embodiment 14      | 384                                                 | 25                   | 0.016                        | 98                               | 25                               | 17.94048                             |
| Embodiment 15      | 384                                                 | 25                   | 0.016                        | 114                              | 25                               | 21.87264                             |
| Embodiment 16      | 385                                                 | 20                   | 0.01                         | 110                              | 25                               | 16.3625                              |
| Embodiment 17      | 382                                                 | 20                   | 0.017                        | 98                               | 25                               | 23.7031                              |
| Embodiment 18      | 383                                                 | 30                   | 0.012                        | 99                               | 25                               | 11.3368                              |
| Embodiment 19      | 384                                                 | 20                   | 0.016                        | 105                              | 25                               | 24.576                               |
| Embodiment 20      | 382                                                 | 20                   | 0.013                        | 106                              | 25                               | 20.1123                              |

40

Table 3 is the performance data of the carriers of the thick film elements in Embodiments 1 to 20. The details are as follows:

TABLE 3

| Carrier       |                                                     |                      |                                  |                                                          |                                  |                                    |
|---------------|-----------------------------------------------------|----------------------|----------------------------------|----------------------------------------------------------|----------------------------------|------------------------------------|
|               | Heat Conductivity Coefficient $\lambda_3$ (W/m · k) | Thickness $d_3$ (μm) | Surface Temperature $T_3$ (° C.) | $T_{\text{Minimum melting point of the carrier}}$ (° C.) | Initial Temperature $T_0$ (° C.) | Heat Transfer Rate/10 <sup>6</sup> |
| Embodiment 1  | 2.2                                                 | 4000                 | 45                               | 350                                                      | 25                               | 0.000132                           |
| Embodiment 2  | 2.1                                                 | 5000                 | 46                               | 350                                                      | 25                               | 0.00010584                         |
| Embodiment 3  | 2.02                                                | 5500                 | 45                               | 350                                                      | 25                               | 8.81455E-05                        |
| Embodiment 4  | 3.4                                                 | 6000                 | 46                               | 350                                                      | 25                               | 0.0001428                          |
| Embodiment 5  | 2.5                                                 | 5800                 | 48                               | 350                                                      | 25                               | 9.91379E-05                        |
| Embodiment 6  | 1.5                                                 | 7000                 | 45                               | 350                                                      | 25                               | 4.28571E-05                        |
| Embodiment 7  | 1.8                                                 | 10000                | 46                               | 350                                                      | 25                               | 0.00005292                         |
| Embodiment 8  | 1.9                                                 | 9000                 | 48                               | 350                                                      | 25                               | 6.79778E-05                        |
| Embodiment 9  | 2.1                                                 | 8800                 | 48                               | 350                                                      | 25                               | 7.68409E-05                        |
| Embodiment 10 | 1.85                                                | 9500                 | 50                               | 350                                                      | 25                               | 5.84211E-05                        |
| Embodiment 11 | 2                                                   | 10500                | 50                               | 350                                                      | 25                               | 5.71429E-05                        |
| Embodiment 12 | 2.01                                                | 6000                 | 52                               | 350                                                      | 25                               | 0.00010854                         |
| Embodiment 13 | 1.8                                                 | 7000                 | 49                               | 350                                                      | 25                               | 7.40571E-05                        |
| Embodiment 14 | 1.89                                                | 8000                 | 48                               | 350                                                      | 25                               | 0.00008694                         |
| Embodiment 15 | 1.78                                                | 9500                 | 50                               | 350                                                      | 25                               | 7.49474E-05                        |
| Embodiment 16 | 2.01                                                | 11000                | 52                               | 350                                                      | 25                               | 4.93364E-05                        |
| Embodiment 17 | 2.34                                                | 7800                 | 51                               | 350                                                      | 25                               | 0.0001326                          |

TABLE 3-continued

|               | Carrier                                                      |                         |                                       |                                                            |                            |                                       |  |
|---------------|--------------------------------------------------------------|-------------------------|---------------------------------------|------------------------------------------------------------|----------------------------|---------------------------------------|--|
|               | Heat<br>Conductivity<br>Coefficient $\lambda_3$<br>(W/m · k) | Thickness<br>$d_3$ (μm) | Surface<br>Temperature<br>$T_3$ (°C.) | $T_{\text{Minimum melting point of the carrier}}$<br>(°C.) | Initial                    |                                       |  |
|               |                                                              |                         |                                       |                                                            | Temperature<br>$T_0$ (°C.) | Heat Transfer<br>Rate/10 <sup>6</sup> |  |
| Embodiment 18 | 2.03                                                         | 8500                    | 48                                    | 350                                                        | 25                         | 6.59153E-05                           |  |
| Embodiment 19 | 1.95                                                         | 9500                    | 47                                    | 350                                                        | 25                         | 7.22526E-05                           |  |
| Embodiment 20 | 1.84                                                         | 5600                    | 47                                    | 350                                                        | 25                         | 9.39714E-05                           |  |

Table 4 is the heat transfer rates calculated according to the performance data listed in Tables 1, 2 and 3. The heat transfer rates of the covering layer, the thick film coating and the carrier are calculated by ratio to obtain the limiting conditions of the material of the present invention, namely the following equations:

$$\lambda_1 A \frac{T_1 - T_0}{d_1} = a \times \lambda_3 A \frac{T_3 - T_0}{d_3},$$

$$\lambda_2 A \frac{T_2 - T_0}{d_2} = b \times \lambda_1 A \frac{T_1 - T_0}{d_1}, \quad \lambda_2 A \frac{T_2 - T_0}{d_2} = c \times \lambda_3 A \frac{T_3 - T_0}{d_3},$$

wherein  $200 \leq a \leq 10^4$ ,  $0 < b \leq 1000$ ,  $0 < c \leq 5 \times 10^5$ .

TABLE 4

| Covering<br>Layer<br>Heat<br>Transfer<br>Rate | Thick Film                            |                                  |             | a         | b         | c         | Satisfy the<br>equations? |  |  |  |  |
|-----------------------------------------------|---------------------------------------|----------------------------------|-------------|-----------|-----------|-----------|---------------------------|--|--|--|--|
|                                               | Coating<br>Heat<br>Generating<br>Rate | Carrier<br>Heat Transfer<br>Rate |             |           |           |           |                           |  |  |  |  |
|                                               |                                       |                                  |             |           |           |           |                           |  |  |  |  |
| Embodiment 1                                  | 36822                                 | 14322000                         | 132         | 278.95455 | 388.95226 | 108500    | Yes                       |  |  |  |  |
| Embodiment 2                                  | 73746                                 | 13977600                         | 105.84      | 696.76871 | 189.53706 | 132063.49 | Yes                       |  |  |  |  |
| Embodiment 3                                  | 90138                                 | 13224000                         | 88.14545455 | 1022.6052 | 146.70838 | 150024.75 | Yes                       |  |  |  |  |
| Embodiment 4                                  | 83622                                 | 9626400                          | 142.8       | 585.58824 | 115.11803 | 67411.765 | Yes                       |  |  |  |  |
| Embodiment 5                                  | 90500                                 | 5882800                          | 99.13793103 | 912.86957 | 65.003315 | 59339.548 | Yes                       |  |  |  |  |
| Embodiment 6                                  | 87356.66667                           | 6758888.889                      | 42.85714286 | 2038.3222 | 77.371186 | 157707.41 | Yes                       |  |  |  |  |
| Embodiment 7                                  | 154800.8                              | 8134000                          | 52.92       | 2925.1852 | 52.544948 | 153703.7  | Yes                       |  |  |  |  |
| Embodiment 8                                  | 150570                                | 13224000                         | 67.97777778 | 2214.9886 | 87.82626  | 194534.16 | Yes                       |  |  |  |  |
| Embodiment 9                                  | 189787.5                              | 10220622.22                      | 76.84090909 | 2469.8758 | 53.852979 | 133010.17 | Yes                       |  |  |  |  |
| Embodiment 10                                 | 167013                                | 10657800                         | 58.42105263 | 2858.7811 | 63.814194 | 182430.81 | Yes                       |  |  |  |  |
| Embodiment 11                                 | 157680                                | 10608685.71                      | 57.14285714 | 2759.4    | 67.279843 | 185652    | Yes                       |  |  |  |  |
| Embodiment 12                                 | 204891.4286                           | 11595428.57                      | 108.54      | 1887.7043 | 56.593039 | 106830.92 | Yes                       |  |  |  |  |
| Embodiment 13                                 | 159342.8571                           | 18924000                         | 74.05714286 | 2151.6204 | 118.76278 | 255532.41 | Yes                       |  |  |  |  |
| Embodiment 14                                 | 212457.1429                           | 17940480                         | 86.94       | 2443.7214 | 84.442819 | 206354.73 | Yes                       |  |  |  |  |
| Embodiment 15                                 | 290218.6667                           | 21872640                         | 74.94736842 | 3872.2996 | 75.366069 | 291840    | Yes                       |  |  |  |  |
| Embodiment 16                                 | 181000                                | 16362500                         | 49.33636364 | 3668.6936 | 90.400552 | 331651.93 | Yes                       |  |  |  |  |
| Embodiment 17                                 | 262570.6667                           | 23703100                         | 132.6       | 1980.1709 | 90.273222 | 178756.41 | Yes                       |  |  |  |  |
| Embodiment 18                                 | 223704                                | 11336800                         | 65.91529412 | 3393.8102 | 50.677681 | 171990.43 | Yes                       |  |  |  |  |
| Embodiment 19                                 | 318835.2                              | 24576000                         | 72.25263158 | 4412.7832 | 77.080573 | 340139.86 | Yes                       |  |  |  |  |
| Embodiment 20                                 | 314431                                | 20112300                         | 93.97142857 | 3346.0277 | 63.964113 | 214025.69 | Yes                       |  |  |  |  |

The results listed in Table 4 show that the thick films prepared according to Embodiments 1 to 20 all satisfy the equations; and the carrier, i.e. covering layer, has the function of generating heat and the temperature difference between two sides are more than 40° C., so as to achieve the function of heat generation. When in use, the product could reduce heat loss when the covering layer of the thick film

60 element is heated, and the temperature could rise to more than 100° C. after giving electricity for two minutes, which demonstrates that the thick film element of the present invention has high heat generation efficiency.

65 Tables 5 to 8 are the performance data of the thick film elements in contrasting examples 1 to 10 of the present

invention. All the performance data is measured as those shown in Tables 1 to 4. The details are as follows:

TABLE 5

| Covering Layer         |                                                     |                      |                                  |                                                                 |                                    |                                    |
|------------------------|-----------------------------------------------------|----------------------|----------------------------------|-----------------------------------------------------------------|------------------------------------|------------------------------------|
|                        | Heat Conductivity Coefficient $\lambda_1$ (W/m · k) | Thickness $d_1$ (μm) | Surface Temperature $T_1$ (° C.) | $T_{\text{Minimum melting point of the covering layer}}$ (° C.) | Initial Temperature $T_0$ (° C. m) | Heat Transfer Rate/10 <sup>6</sup> |
| Contrasting Example 1  | 7.21                                                | 80                   | 42                               | 350                                                             | 25                                 | 0.02757825                         |
| Contrasting Example 2  | 7.21                                                | 80                   | 43                               | 350                                                             | 25                                 | 0.0292005                          |
| Contrasting Example 3  | 7.22                                                | 100                  | 92                               | 350                                                             | 25                                 | 0.0870732                          |
| Contrasting Example 4  | 7.22                                                | 100                  | 91                               | 350                                                             | 25                                 | 0.0810084                          |
| Contrasting Example 5  | 7.18                                                | 200                  | 46                               | 350                                                             | 25                                 | 0.0128163                          |
| Contrasting Example 6  | 7.18                                                | 200                  | 94                               | 350                                                             | 25                                 | 0.0644046                          |
| Contrasting Example 7  | 7.15                                                | 500                  | 45                               | 350                                                             | 25                                 | 0.007436                           |
| Contrasting Example 8  | 7.22                                                | 500                  | 100                              | 350                                                             | 25                                 | 0.058482                           |
| Contrasting Example 9  | 7.22                                                | 600                  | 42                               | 350                                                             | 25                                 | 0.0110466                          |
| Contrasting Example 10 | 7.24                                                | 600                  | 91                               | 350                                                             | 25                                 | 0.0430056                          |

TABLE 6

| Thick Film Coating     |                                                     |                      |                              |                                  |                                  |                                      |
|------------------------|-----------------------------------------------------|----------------------|------------------------------|----------------------------------|----------------------------------|--------------------------------------|
|                        | Heat Conductivity Coefficient $\lambda_2$ (W/m · k) | Thickness $d_2$ (μm) | Area $A_2$ (m <sup>2</sup> ) | Heating temperature $T_2$ (° C.) | Initial temperature $T_0$ (° C.) | Heat Generating Rate/10 <sup>6</sup> |
| Contrasting Example 1  | 382                                                 | 22                   | 0.018                        | 48                               | 25                               | 7.188545455                          |
| Contrasting Example 2  | 382                                                 | 22                   | 0.018                        | 52                               | 25                               | 8.438727273                          |
| Contrasting Example 3  | 382                                                 | 25                   | 0.018                        | 98                               | 25                               | 20.07792                             |
| Contrasting Example 4  | 382                                                 | 25                   | 0.017                        | 96                               | 25                               | 18.44296                             |
| Contrasting Example 5  | 382                                                 | 30                   | 0.017                        | 48                               | 25                               | 4.978733333                          |
| Contrasting Example 6  | 382                                                 | 30                   | 0.026                        | 101                              | 25                               | 25.16106667                          |
| Contrasting Example 7  | 382                                                 | 32                   | 0.026                        | 49                               | 25                               | 7.449                                |
| Contrasting Example 8  | 382                                                 | 32                   | 0.054                        | 104                              | 25                               | 50.925375                            |
| Contrasting Example 9  | 382                                                 | 35                   | 0.054                        | 46                               | 25                               | 12.3768                              |
| Contrasting Example 10 | 382                                                 | 35                   | 0.054                        | 98                               | 25                               | 43.02411429                          |

TABLE 7

| Carrier               |                                                     |                      |                                  |                                                          |                                  |                                    |
|-----------------------|-----------------------------------------------------|----------------------|----------------------------------|----------------------------------------------------------|----------------------------------|------------------------------------|
|                       | Heat Conductivity Coefficient $\lambda_3$ (W/m · k) | Thickness $d_3$ (mm) | Surface Temperature $T_3$ (° C.) | $T_{\text{Minimum melting point of the carrier}}$ (° C.) | Initial temperature $T_0$ (° C.) | Heat Transfer Rate/10 <sup>3</sup> |
| Contrasting Example 1 | 7.18                                                | 2000                 | 41                               | 350                                                      | 25                               | 0.00103392                         |
| Contrasting Example 2 | 7.18                                                | 2500                 | 37                               | 350                                                      | 25                               | 0.000620352                        |

TABLE 7-continued

|                        | Carrier                                             |                      |                                  |                                                          |                                  |                                    |
|------------------------|-----------------------------------------------------|----------------------|----------------------------------|----------------------------------------------------------|----------------------------------|------------------------------------|
|                        | Heat Conductivity Coefficient $\lambda_3$ (W/m · k) | Thickness $d_3$ (mm) | Surface Temperature $T_3$ (° C.) | $T_{\text{Minimum melting point of the carrier}}$ (° C.) | Initial temperature $T_0$ (° C.) | Heat Transfer Rate/10 <sup>3</sup> |
| Contrasting Example 3  | 7.18                                                | 3600                 | 77                               | 350                                                      | 25                               | 0.0018668                          |
| Contrasting Example 4  | 7.21                                                | 1100                 | 86                               | 350                                                      | 25                               | 0.006797064                        |
| Contrasting Example 5  | 7.21                                                | 1800                 | 41                               | 350                                                      | 25                               | 0.001089511                        |
| Contrasting Example 6  | 7.21                                                | 2800                 | 84                               | 350                                                      | 25                               | 0.00395005                         |
| Contrasting Example 7  | 7.19                                                | 3500                 | 35                               | 350                                                      | 25                               | 0.000534114                        |
| Contrasting Example 8  | 7.19                                                | 3200                 | 88                               | 350                                                      | 25                               | 0.007643869                        |
| Contrasting Example 9  | 7.19                                                | 3800                 | 32.5                             | 350                                                      | 25                               | 0.000766303                        |
| Contrasting Example 10 | 7.2                                                 | 100                  | 91.5                             | 350                                                      | 25                               | 0.258552                           |

TABLE 8

| Covering Layer Heat Transfer Rate | Thick Film Coating Heat Generating Rate | Carrier Heat Transfer Rate | a           | b         | c         | Satisfy the equations? |
|-----------------------------------|-----------------------------------------|----------------------------|-------------|-----------|-----------|------------------------|
|                                   |                                         |                            |             |           |           |                        |
| Contrasting Example 1             | 27578.25                                | 7188545.455                | 1033.92     | 26.673485 | 260.65996 | 6952.7095              |
| Contrasting Example 2             | 29200.5                                 | 8438727.273                | 620.352     | 47.070857 | 288.99256 | 13603.127              |
| Contrasting Example 3             | 87073.2                                 | 20077920                   | 1866.8      | 46.643025 | 230.58668 | 10755.26               |
| Contrasting Example 4             | 81008.4                                 | 18442960                   | 6797.063636 | 11.918146 | 227.66725 | 2713.3717              |
| Contrasting Example 5             | 12816.3                                 | 4978733.333                | 1089.511111 | 11.76335  | 388.46885 | 4569.6949              |
| Contrasting Example 6             | 64404.6                                 | 25161066.67                | 3950.05     | 16.304756 | 390.67189 | 6369.8097              |
| Contrasting Example 7             | 7436                                    | 7449000                    | 534.1142857 | 13.922114 | 1001.7483 | 13946.453              |
| Contrasting Example 8             | 58482                                   | 50925375                   | 7643.86875  | 7.6508378 | 870.78717 | 6662.2514              |
| Contrasting Example 9             | 11046.6                                 | 12376800                   | 766.3026316 | 14.415454 | 1120.4171 | 16151.321              |
| Contrasting Example 10            | 43005.6                                 | 43024114.29                | 258552      | 0.1663325 | 1000.4305 | 166.40411              |

Material and structure of the thick film elements in the Contrasting Examples 1 to 10 listed in the above tables neither meet the material selection requirement of the present invention, nor satisfy the equations of the present invention. After given electricity and heat generation, the temperatures difference between the two sides of the thick film elements of the Contrasting Examples 1 to 10 are not significantly different, and the heating temperature difference between the covering layer and the carrier is smaller than 15° C. . The thick film elements prepared according to such material selections do not meet the requirement of the thick film element having a covering layer with high heat conductivity of the present invention or meet the product requirement of the present invention, which demonstrates the heat transfer rate and correlation of the present invention.

When the thick film elements of the Embodiments 1 to 20 is applied in winter clothes, the side of the covering layer that transfers heat is set adjacent to the direction of the human body, and the carrier of the thick film element is set

away from the human body. When given electricity to generate heat, only the covering layer of the thick film element produces heat. The thick film element having a covering layer with high heat conductivity has the following advantageous effects: (1) only the covering layer transfers heat, and requirement for heat conduction performance of the carrier is not strict, which allows a wide range of materials to be selected as the coated substrate of the thick film; (2) the covering layer of the thick film element is required to be very thin, which makes the thick film element much smaller, more exquisite and more light weighted and allows the wearer to feel more comfortable when the thick film is placed in clothes; (3) when the thick film element is applied in clothes, it is only required that the side facing the human body transfers heat, and there is no need for the opposite side to transfer heat, which could avoid filling of thermal isolation materials at the opposite side and could reduce heat loss. In contrast, heat transferring effect between the two sides of the thick film elements in the contrasting

examples is not significantly different; when applied in the clothes with a single-side heat transferring covering layer, the thick film elements would cause heat loss and filling thermal isolation materials at the opposite side would be required, thus increasing the cost and weight of the clothes and reducing comfort of the wearer.

According to the disclosure and teaching of above-mentioned specification, those skilled in the art of the present invention can still make changes and modifications to above-mentioned embodiment, therefore, the scope of the present invention is not limited to the specific embodiments disclosed and described above, and all those modifications and changes to the present invention are within the scope of the present invention as defined in the appended claims. Besides, although some specific terminologies are used in the specification, it is merely as a clarifying example and shall not be construed as limiting the scope of the present invention in any way.

What is claimed is:

1. A thick film element having a covering layer with high heat conductivity, comprising: a carrier; a thick film coating deposited on the carrier; and a covering layer overlaid on the coating, wherein the thick film coating is a heating material, and a mode of heating is electrical heating, wherein the carrier, the thick film coating and the covering layer are selected from a material that fulfills every of following equations:

$$\lambda_1 A \frac{T_1 - T_0}{d_1} = a \times \lambda_3 A \frac{T_3 - T_0}{d_3},$$

$$\lambda_2 A \frac{T_2 - T_0}{d_2} = b \times \lambda_1 A \frac{T_1 - T_0}{d_1}, \quad \lambda_2 A \frac{T_2 - T_0}{d_2} = c \times \lambda_3 A \frac{T_3 - T_0}{d_3};$$

wherein  $200 \leq a \leq 10^4$ ,  $0 < b \leq 1000$ ,  $0 < c \leq 5 \times 10^5$ ;

$T_2 < T_{\text{Minimum melting point of the covering layer}}$ ;

$T_2 < T_{\text{Minimum melting point of the carrier}}$ ;

$T_0 \leq 30^\circ \text{C}$ ;

wherein a value of

$$\lambda_1 A \frac{T_1 - T_0}{d_1}$$

represents a heat transfer rate of the covering layer; a value of

$$\lambda_2 A \frac{T_2 - T_0}{d_2}$$

represents a heat generating rate of the thick film coating; a value of

$$\lambda_3 A \frac{T_3 - T_0}{d_3}$$

represents a heat transfer rate of the carrier;

$\lambda_1$  represents a heat conductivity coefficient of the covering layer at a temperature of  $T_1$ ;

$\lambda_2$  represents a heat conductivity coefficient of the thick film coating at a temperature of  $T_2$ ;

$\lambda_3$  represents a heat conductivity coefficient of the carrier at a temperature of  $T_3$ ;

$A$  represents a contact area of the thick film coating with the covering layer or the carrier;

$d_1$  represents a thickness of the covering layer;

$d_2$  represents a thickness of the thick film coating;

$d_3$  represents a thickness of the carrier;

$T_0$  represents an initial temperature of the thick film heating element;

$T_1$  represents a surface temperature of the covering layer;

$T_2$  represents a heating temperature of the thick film coating;

$T_3$  represents a surface temperature of the carrier;

$d_2 \leq 50 \mu\text{m}$ ;  $10 \mu\text{m} \leq d_1 \leq 10 \text{ mm}$ ,  $d_3 \geq 10 \mu\text{m}$ ;

$T > 25^\circ \text{C}$ ; and  $\lambda_1 \geq \lambda_3$ .

2. The thick film element according to claim 1, wherein the heat conductivity coefficient  $\lambda_3$  of the carrier is smaller than or equal to  $3 \text{ W/m}\cdot\text{k}$ , the heat conductivity coefficient  $\lambda_1$  of the covering layer is larger than or equal to  $3 \text{ W/m}\cdot\text{k}$ , and  $200 \leq a \leq 10^4$ ,  $10 \leq b \leq 1000$ ,  $10^4 \leq c \leq 5 \times 10^5$ .

3. The thick film element according to claim 2, wherein a region between the carrier and the covering layer without the thick film coating is bound by printing, coating, spraying or sintering, or gluing.

4. The thick film element according to claim 1, wherein the carrier and the thick film coating are bound by printing or sintering, and the thick film coating and the covering layer are bound by printing, sintering, or vacuum.

5. The thick film element according to claim 1, wherein the carrier comprises polyimides, organic insulating materials, inorganic insulating materials, ceramics, glass ceramics, quartz, stone materials, fabrics and fiber.

6. The thick film element according to claim 1, wherein the thick film coating is one or more of silver, platinum, palladium, palladium oxide, gold and rare earth materials.

7. The thick film element according to claim 1, wherein the covering layer is made from one or more of polyester, polyimide or polyetherimide (PEI), ceramics, silica gel, asbestos, micarex, fabric and fiber.

8. The thick film element according to claim 1, wherein an area of the thick film coating is smaller than or equal to an area of the covering layer or an area of the carrier.

9. An use of a thick film element for coating products having a single-sided heating covering layer, wherein the thick film element has a covering layer with high heat conductivity and comprises: a carrier; a thick film coating deposited on the carrier; and a covering layer overlaid on the coating, wherein the thick film coating is a heating material, and a mode of heating is electrical heating, wherein the carrier, the thick film coating and the covering layer are selected from a material that fulfills every of following equations:

50

$$\lambda_1 A \frac{T_1 - T_0}{d_1} = a \times \lambda_3 A \frac{T_3 - T_0}{d_3},$$

$$\lambda_2 A \frac{T_2 - T_0}{d_2} = b \times \lambda_1 A \frac{T_1 - T_0}{d_1}, \quad \lambda_2 A \frac{T_2 - T_0}{d_2} = c \times \lambda_3 A \frac{T_3 - T_0}{d_3};$$

55

wherein  $200 \leq a \leq 10^4$ ,  $0 < b \leq 1000$ ,  $0 < c \leq 5 \times 10^5$ ;

$T_2 < T_{\text{Minimum melting point of the covering layer}}$ ;

$T_2 < T_{\text{Minimum melting point of the carrier}}$ ;

$T_0 \leq 30^\circ \text{C}$ ;

wherein a value of

$$\lambda_1 A \frac{T_1 - T_0}{d_1}$$

65

**19**

represents a heat transfer rate of the covering layer;  
a value of

$$\lambda_2 A \frac{T_2 - T_0}{d_2}$$

represents a heat generating rate of the thick film coating;  
a value of

$$\lambda_3 A \frac{T_3 - T_0}{d_3}$$

represents a heat transfer rate of the carrier;

$\lambda_1$  represents a heat conductivity coefficient of the covering layer at a temperature of  $T_1$ ;

$\lambda_2$  represents a heat conductivity coefficient of the thick film coating at a temperature of  $T_2$ ;

$\lambda_3$  represents a heat conductivity coefficient of the carrier at a temperature of  $T_3$ ;

$A$  represents a contact area of the thick film coating with the covering layer or the carrier;

$d_1$  represents a thickness of the covering layer;

$d_2$  represents a thickness of the thick film coating;

$d_3$  represents a thickness of the carrier;

$T_0$  represents an initial temperature of the thick film heating element;

$T_1$  represents a surface temperature of the covering layer;

$T_2$  represents a heating temperature of the thick film coating;

$T_3$  represents a surface temperature of the carrier;

**20**

$d_2 \leq 50 \mu\text{m}$ ;  $10 \mu\text{m} \leq d_1 \leq 10 \text{ mm}$ ,  $d_3 \geq 10 \mu\text{m}$ ;  
 $T_{\text{Minimum melting point of the carrier}} > 25^\circ \text{C}$ ; and  $\lambda_1 > \lambda_3$ .

**10.** The use of the thick film element according to claim 9, wherein the heat conductivity coefficient  $\lambda_3$  of the carrier is smaller than or equal to 3 W/m·k, the heat conductivity coefficient  $\lambda_1$  of the covering layer is larger than or equal to 3 W/m·k, and  $200 \leq a \leq 10^4$ ,  $10 \leq b \leq 1000$ ,  $10^4 \leq c \leq 5 \times 10^5$ .

**11.** The use of the thick film element according to claim 10, wherein a region between the carrier and the covering layer without the thick film coating is bound by printing, coating, spraying or sintering, or gluing.

**12.** The use of the thick film element according to claim 9, wherein the carrier and the thick film coating are bound by printing or sintering, and the thick film coating and the covering layer are bound by printing, sintering, or vacuum.

**13.** The use of the thick film element according to claim 9, wherein the carrier comprises polyimides, organic insulating materials, inorganic insulating materials, ceramics, glass ceramics, quartz, stone materials, fabrics and fiber.

**14.** The use of the thick film element according to claim 9, wherein the thick film coating is one or more of silver, platinum, palladium, palladium oxide, gold and rare earth materials.

**15.** The use of the thick film element according to claim 9, wherein the covering layer is made from one or more of polyester, polyimide or polyetherimide (PEI), ceramics, silica gel, asbestos, micarex, fabric and fiber.

**16.** The use of the thick film element according to claim 9, wherein an area of the thick film coating is smaller than or equal to an area of the covering layer or an area of the carrier.

\* \* \* \* \*